

March 25, 1941.

R. L. FREEMAN

2,235,816

VACUUM TUBE WITH SUBSTANTIALLY CONSTANT INTERELECTRODE CAPACITANCE

Filed Oct. 14, 1939



FIG. 1.

Dielectric Material with Negative  
Coefficient of Permittivity.



FIG. 2.

Dielectric Material with Negative  
Coefficient of Permittivity.

INVENTOR  
ROBERT L. FREEMAN

BY *Lawrence B. Dodds*  
ATTORNEY

## UNITED STATES PATENT OFFICE

2,235,816

## VACUUM TUBE WITH SUBSTANTIALLY CONSTANT INTERELECTRODE CAPACITANCE

Robert L. Freeman, Flushing, N. Y., assignor to Hazeltine Corporation, a corporation of Delaware

Application October 14, 1939, Serial No. 299,430

6 Claims. (Cl. 250—27.5)

This invention relates generally to vacuum tubes and particularly to vacuum tubes designed for operation in ultra-high-frequency modulated-carrier signal-translating systems. A tube incorporating the principles of the invention is of particular utility for use in the circuit of the local oscillator of an ultra-high-frequency receiver of the superheterodyne type.

In some vacuum-tube signal-translating systems, the interelectrode capacitance of the vacuum tubes utilized is appreciable and must be taken into account in the circuit design. This is particularly true in systems for operation at ultra-high frequencies for the reason that in such systems the interelectrode capacitance of the vacuum tubes utilized is a very appreciable portion of the total circuit capacitance. The interelectrode capacitances of all conventional tubes are influenced to some extent by temperature and such capacitance changes occurring during the warm-up period of a particular system may be very disadvantageous. A concrete example may be taken as the local oscillator tube in a television receiver of the superheterodyne type. The oscillator for such a receiver generally operates at such a high frequency that the interelectrode capacitance is an appreciable part of the total capacitance of the frequency-determining circuit of the oscillator. Thus, as such a receiver warms up after being placed in operation, the interelectrode capacitance of the oscillator tube may change to such an extent as to vary the oscillator frequency by as much as 200 kilocycles. Obviously, such a change in the local oscillator frequency may seriously impair the quality of reproduction, particularly in the sound-signal channel. These interelectrode capacitance changes of the local oscillator tube are probably due principally to (1) variations in geometrical capacitance occasioned by thermal expansion of tube elements and of the envelope, if a conductive envelope is utilized, and (2) changes in the dielectric constant of the various insulating materials utilized in the tube's construction.

It is an object of the invention, therefore, to provide an improved vacuum tube not subject to the above-mentioned disadvantage of vacuum tubes of the prior art.

It is another object of the invention to provide an improved vacuum tube in which the interelectrode capacitances remain substantially constant irrespective of variations in the operating temperature of the tube.

In accordance with the invention, a vacuum

tube comprises an envelope, a plurality of electrodes mounted therein, lead-in wires for the electrodes extending through the tube envelope, certain of the electrodes having therebetween undesired capacitance which tends to vary positively with temperature during normal operation, and dielectric material effectively having a negative temperature coefficient of permittivity separating the lead-in wires of said certain electrodes and disposed to be heated by the other elements of the vacuum tube during normal operation thereof, the configuration of the dielectric material and its temperature coefficient of permittivity being relatively so proportioned that variations of said undesired capacitance are compensated by variations in the permittivity of the dielectric material.

In a preferred embodiment of the invention the envelope is of metal and the configuration of the dielectric material and the area thereof in contact with the envelope of the tube is so proportioned that changes in the interelectrode capacitances due to heating of the dielectric substantially compensate for undesirable changes in interelectrode capacitances between at least certain of the electrodes of the tube.

For a better understanding of the invention, together with other and further objects thereof, reference is had to the following description taken in connection with the accompanying drawing, and its scope will be pointed out in the appended claims.

Each of Figs. 1 and 2 of the drawing is a perspective view of a vacuum tube incorporating the invention with a portion of the envelope broken away.

Referring now more particularly to Fig. 1 of the drawing, there is shown a vacuum tube incorporating the invention which comprises a plurality of electrodes including a cathode 10, a control electrode 11, and an anode 12, all of the electrodes being enclosed within an envelope 13. A suitable heater 14 is provided for cathode 10. Lead-in wires 16 for electrodes 10, 11, and 12 and heater 14 are brought out of the envelope 13 through a button 15 which may be of glass or other suitable insulating material. The envelope 13 may be of metal and the button 15 sealed therewith by means of a metal sealing flange 17. Suitable longitudinal supports 18 are also embedded in button 15 for supporting the various electrodes of the tube, the supports 18 being rigidly held transversely of the tube by an insulating disc 19, preferably of mica, through which they extend. Suitable contact prongs 20 for the

5

10

15

25

30

35

40

45

50

55

vacuum tube are rigidly mounted in a base 21 of dielectric material, which is in intimate contact with the tube envelope 13, and are electrically connected to, and are effectively extensions of, the various lead-in wires 10.

In considering the tube just described, it will be seen that the envelope 13, button 15, and sealing flange 17 are effective to enclose the electrode structure of the tube within a sealed evacuated chamber, in accordance with conventional vacuum-tube practice. Conventional vacuum tubes, however, as brought out in the preliminary part of this specification, and especially those vacuum tubes which are designed for operation in ultra-high-frequency circuits, have between certain of the electrodes appreciable undesired interelectrode capacitances which tend to vary positively with temperature during normal operation of the tube. Such variations of interelectrode capacitances, which are sometimes detrimental in the operation of the circuit in which the tubes are used, may be due to the thermal expansion of metal parts of the tube or may be caused by heating of the various dielectric elements used in the tube, such as button 15, which generally have a positive temperature coefficient of permittivity. In accordance with the present invention, therefore, the base 21, which supports contact prongs 20 and effectively separates the lead-in wires 30 of the tube electrodes, is constructed of a dielectric material having a negative temperature coefficient of permittivity; that is, a dielectric constant which decreases with increase in temperature of the base 21. The configuration of dielectric material or base 21, the area thereof in contact with the envelope 13, and the temperature coefficient of permittivity of the material are relatively so proportioned that the capacitances between contact prongs 20 through dielectric base 21 decrease, due to heat transferred from metal envelope 13 and from other elements of the tube to base 21 during normal operation of the tube, at substantially the same rate as the interelectrode capacitances between the electrodes of the tube increase. Thus, the variations of undesired interelectrode capacitances are compensated by variation in the permittivity of the dielectric material. Since the total or effective interelectrode capacitances of the tube as connected in a circuit are the sums of the capacitances between the electrodes themselves, their lead-in wires, and the contact prongs, the structure of Fig. 1 is effective to provide a tube, the effective interelectrode capacitances of which are substantially constant irrespective of variations of temperature during operation of the tube.

While applicant does not intend to be limited to any particular dielectric material for use in the insulating base 21, the ceramic insulating material known as "Alsimag 190" of the American Lava Corporation, Chattanooga, Tennessee, has particularly desirable characteristics. This material comprises 95 per cent titanium dioxide in the form of rutile crystals developed by firing amorphous titanium dioxide, the remaining 5 per cent being a glassy or partly crystalline material including aluminum oxide ( $Al_2O_3$ ), silicon dioxide ( $SiO_2$ ), and magnesium oxide ( $MgO$ ), and has a temperature coefficient of permittivity between 20 and 80 degrees C of  $-6.5 \times 10^{-4}$  microfarads per microfarad per degree C. Polystyrene resin, which has a temperature coefficient of permittivity of  $-0.35 \times 10^{-4}$  micro-microfarads per micro-micro-farad per degree C., may also be used. A polystyrene resin having such

properties is produced by the Dielectric Products Corporation, Jersey City, N. J., under the trade name of "Victron." This material is a synthetic resin produced by the isolation and subsequent polymerization of the monomeric styrene,  $C_6H_5-CH=CH_2$  and is described in Electrochemical Society Reprint 74-35, page 545. Commercially available "Halowax" also exhibits a negative temperature coefficient of permittivity at ordinary working temperatures of a vacuum tube. Such material might be used to provide a dielectric base, similar to base 21 described above, even though a contact-supporting structure of a ceramic material were also utilized.

While a triode has been illustrated in Fig. 1 for the sake of simplicity, it will be understood that applicant's invention is applicable to vacuum tubes of other electrode structures.

In Fig. 2, there is shown a modified embodiment of the invention which is generally similar to that of Fig. 1 and in which similar circuit elements have identical reference numerals. The tube of Fig. 2 differs from that of Fig. 1 in that it has an envelope 23 of dielectric material and comprises a button or press 24 within which the lead-in wires or contact prongs 20 are sealed. At least a portion of the envelope 23 adjacent the contact prongs 20 is constructed of a dielectric material separating the contact prongs or lead-in wires and disposed to be heated by the other elements of the tube during normal operation thereof. This dielectric material has a negative temperature coefficient of permittivity and its configuration and coefficient of permittivity are relatively so proportioned as to provide capacitance compensation similar to that provided by the base 21 of the tube of Fig. 1. For instance, the envelope 23 may be of glass comprising as an ingredient an appreciable amount of titanium dioxide in order to impart thereto a negative temperature coefficient of permittivity.

It will be understood that the heating of the base 21 of the tube of Fig. 1 and of the press 24 of the tube of Fig. 2 is, to some extent, dependent upon the transfer of heat from contact prongs 20 to the dielectric material therebetween.

While there have been described what are at present considered to be the preferred embodiments of this invention, it will be obvious to those skilled in the art that various changes and modifications may be made therein without departing from the invention, and it is, therefore, aimed in the appended claims to cover all such changes and modifications as fall within the true spirit and scope of the invention.

#### What is claimed is:

1. A vacuum tube comprising, an envelope, a plurality of electrodes mounted therein, lead-in wires for said electrodes extending through said envelope, certain of said electrodes having therebetween undesired capacitance which tends to vary positively with temperature during normal operation, and dielectric material effectively having a negative temperature coefficient of permittivity separating the lead-in wires of said certain electrodes and disposed to be heated by the other elements of said vacuum tube during normal operation thereof the configuration of said dielectric material and its temperature coefficient of permittivity being relatively so proportioned that variations of said undesired capacitance are compensated by variations in the permittivity of said dielectric material.
2. A vacuum tube comprising, an envelope, a plurality of electrodes mounted therein, lead-in

wires for said electrodes extending through said envelope, certain of said electrodes having therebetween undesired capacitance which tends to vary positively with temperature during normal operation, and dielectric material comprising an amount of titanium dioxide sufficient to impart thereto a substantial negative temperature coefficient of permittivity separating the lead-in wires of said certain electrodes and disposed to be heated by the other elements of said vacuum tube during normal operation thereof the configuration of said dielectric material and its temperature coefficient of permittivity being relatively so proportioned that variations of said undesired capacitance are compensated by variations in the permittivity of said dielectric material.

3. A vacuum tube comprising, an envelope, a plurality of electrodes mounted therein, lead-in wires for said electrodes extending through said envelope, contact prongs connected to said lead-in wires, certain of said electrodes having therebetween undesired capacitance which tends to vary positively with temperature during normal operation, and a base of dielectric material separate from said envelope but in intimate contact therewith and having a negative temperature coefficient of permittivity, said base supporting said contact prongs, the configuration of said dielectric material and its temperature coefficient of permittivity being relatively so proportioned that variations of said undesired capacitances are compensated by variations in the permittivity of said dielectric material between the ones of said prongs which are connected to said certain electrodes.

4. A vacuum tube comprising, an envelope, a plurality of electrodes mounted therein, and lead-in wires for said electrodes extending through said envelope, certain of said electrodes having therebetween undesired capacitance which tends to vary positively with temperature during normal operation, said envelope comprising a portion adjacent said lead-in wires having a negative temperature coefficient of permittivity dis-

posed to be heated by the other elements of said vacuum tube during normal operation thereof, the configuration of said envelope portion and said negative temperature coefficient of permittivity being relatively so proportioned that variations of said undesired capacitance are compensated by variations in the permittivity of said dielectric material.

5. A vacuum tube comprising, a metal envelope, a plurality of electrodes mounted therein, lead-in wires for said electrodes, contact prongs connected to said lead-in wires, and a base of dielectric material separate from said envelope and having a negative temperature coefficient of permittivity, said base being in intimate contact with said envelope and supporting said contact prongs, the capacitances between certain of said electrodes being subject to undesired increases due to heating during operation of said tube, and the configuration of said dielectric material and the area thereof in contact with said envelope being so proportioned that the intercontact capacitances through said dielectric material decrease due to heat transferred from said envelope to said base during operation of said tube at substantially the same rate as said undesired capacitance increases.

6. A vacuum tube comprising, an envelope, a plurality of electrodes mounted therein, lead-in wires for said electrodes extending through said envelope, said envelope comprising a portion of dielectric material separating said lead-in wires and disposed to be heated by the other elements of said vacuum tube during normal operation thereof, the capacitances between certain of said electrodes being subject to undesired increases due to heating during operation of said tube, and at least said portion of said dielectric material between said certain electrodes effectively having a negative temperature coefficient of permittivity proportioned substantially to compensate said undesired capacitance increases.

ROBERT L. FREEMAN.